

## UNITED STATES PATENT OFFICE

1,924,722

METHOD AND MEANS FOR REMOVING  
CARBON DEPOSITS

Wheeler G. Lovell and Thomas A. Boyd, Detroit,  
Mich., assignors to General Motors Research  
Corporation, Detroit, Mich., a corporation of  
Delaware

No Drawing. Application August 28, 1929  
Serial No. 389,089

8 Claims. (Cl. 87—5)

This application relates to the removal of carbon deposits from the combustion chambers of internal combustion engines, and its principal objects are to employ compounds particularly suitable for this purpose and a process adapted to employ these compounds at their highest efficiency.

We have found that aliphatic amides such as diethyl formamide and formamide which will remove varnish are particularly useful in removing carbon deposits, and that the best method of using them is to apply them to carbon coated parts which have been heated preferably to a temperature above 150° F., the optimum conditions for water cooled engines being at approximately the boiling point of water. We may also use with aliphatic amides a mixture of benzol and alcohol, or other low boiling varnish remover, which apparently increases the solvent action of aliphatic amides not only by reducing the viscosity, but also because they are lower boiling and tend to keep the liquid in contact with the carbon in a mild state of agitation.

As a specific example we may use in each cylinder of an ordinary six cylinder engine 30 c.c. of a mixture comprising by volume 20 parts of diethyl formamide, 40 parts of benzol, and 40 parts of ethyl alcohol. The engine is operated until the temperature of the metal parts of the combustion chamber is at least 150° F. when the mixture is injected or otherwise introduced into the cylinders and the engine stopped. The mixture is permitted to remain in the cylinders for about two hours, more or less, depending upon the nature of the carbon deposit, during which time the gummy binder is softened or dissolved. Then the engine is started and the loosened deposit is gradually blown out the exhaust.

When cleaning the parts by hand they may be heated, the solvent applied, and when the binder is softened the deposit may be wiped off.

It is within the scope of the present invention to employ any aliphatic amide which is a varnish remover and to vary the proportions according to the compound used and the specific conditions, and the aliphatic amide may be used alone.

We claim:—

1. The process of removing carbon deposits from the combustion chamber of an internal combustion engine which comprises applying to the carbon deposit an aliphatic amide which removes varnish, and removing the carbon deposit.
2. The process of removing carbon deposits from the combustion chamber of an internal combustion engine which comprises applying to

the carbon deposit diethyl formamide, and removing the carbon deposit.

3. The process of removing carbon deposits from the combustion chamber of an internal combustion engine which comprises heating the 60 coated parts, applying to the carbon deposit an aliphatic amide which removes varnish, and a low boiling varnish remover, and removing the carbon deposit.

4. The process of removing carbon deposits 65 from the combustion chamber of an internal combustion engine which comprises heating the coated parts to above 150° F., applying to the carbon deposit an aliphatic amide which removes varnish, benzol and alcohol, and removing the 70 carbon deposit.

5. The process of removing carbon deposits from the combustion chamber of an internal combustion engine which comprises heating the 75 coated parts, applying to the carbon deposit diethyl formamide, benzol and alcohol, and removing the carbon deposit.

6. The process of removing carbon deposits from the combustion chamber of an internal combustion engine which comprises heating the 80 coated parts to above 150° F., applying to the carbon deposit diethyl formamide, benzol and alcohol, and removing the carbon deposit.

7. A composition of matter for removing carbon deposits from internal combustion engines 85 comprising an aliphatic amide which removes varnish, and a low boiling varnish remover.

8. A composition of matter for removing carbon deposits from internal combustion engines comprising diethyl formamide, benzol and 90 alcohol.

WHEELER G. LOVELL.  
THOMAS A. BOYD.

95

100

105

110